

# United States Patent

[19]

[11] 3,926,548

Moriyama et al.

[45] Dec. 16, 1975

[54] **SULFONATED  
PHENYLAMINO-HALOTRIAZINE OR-  
DIAZINE SURFACE MODIFIED AMINATED  
HYDROPHOBIC FIBERS AND BLENDS  
THEREOF WITH UNMODIFIED AMINATED  
HYDROPHOBIC FIBERS**

[75] Inventors: **Kazuo Moriyama; Takashi Iwato;  
Morihiro Ohno, all of Takatsuki,  
Japan**

[73] Assignee: **Toyo Boseki Kabushiki Kaisha,  
Osaka, Japan**

[22] Filed: **Oct. 10, 1972**

[21] Appl. No.: **296,207**

[30] **Foreign Application Priority Data**

Oct. 8, 1971 Japan ..... 46-79786

[52] **U.S. Cl. .... 8/115.5; 8/15; 8/65;  
8/DIG. 21; 8/168; 28/72.12; 28/74 R; 8/115**

[51] **Int. Cl.<sup>2</sup> ..... D06P 5/12**

[58] **Field of Search ..... 8/15, 65, 115.5, DIG. 21,  
8/168 B; 28/74, 72.12**

[56] **References Cited**

UNITED STATES PATENTS

|           |         |                  |           |
|-----------|---------|------------------|-----------|
| 1,886,480 | 11/1972 | Haller .....     | 8/14      |
| 3,083,118 | 3/1963  | Bridgeford ..... | 8/127.6 X |
| 3,481,682 | 12/1969 | Machell .....    | 8/15      |
| 3,632,291 | 1/1972  | Defago .....     | 8/25      |
| 3,775,045 | 11/1973 | Buehler .....    | 8/15      |

*Primary Examiner*—Donald Levy

*Attorney, Agent, or Firm*—Wenderoth, Lind & Ponack

[57] **ABSTRACT**

Hydrophobic fibers containing amino groups and having a dye-reserved surface so as to render the fibers non-dyeable or differential-dyeable, and a process for their preparation.

**9 Claims, 2 Drawing Figures**



Fig. 1



Fig. 2



SULFONATED PHENYLAMINO-HALOTRIAZINE OR-DIAZINE SURFACE MODIFIED AMINATED HYDROPHOBIC FIBERS AND BLENDS THEREOF WITH UNMODIFIED AMINATED HYDROPHOBIC FIBERS

The present invention relates to hydrophobic fibers containing amino groups of which only the surface layer is processed so as to be dye-reserving to render the fibers non-dyeable or differential-dyeable and also to a process for producing the same.

An object of the present invention is to provide hydrophobic fibers containing amino groups, which are non-dyeable or differential-dyeable with anionic dyes.

Another object of the present invention is to provide hydrophobic fibers containing amino groups which are differential-dyeable with the use of only anionic dyes.

A further object of the present invention is to provide a process for producing the above-mentioned hydrophobic fibers containing amino groups which are non-dyeable or differential-dyeable.

The invention will be explained in detail as follows by referring partly to the accompanying drawings wherein FIG. 1 is a schematic cross-section of a fiber embodying this invention and FIG. 2 is a schematic longitudinal sectional view of an apparatus useful for producing the fibers of this invention.

Referring to FIG. 1 which is a schematic cross-section of a single fiber of the present invention, the numeral 1 indicates a layer which has been processed to be dye-reserving to make the fiber non-dyeable or differential-dyeable (hereinafter referred to as dye-reserving layer, for simplicity) and the numeral 2 designates an ordinary dye-acceptable core portion of the fiber.

The hydrophobic fiber of the present invention preferably has a dye-reserving layer of a thickness of less than 2 microns on the average. As the thickness of the surface dye-reserving layer exceeds 2 microns on the average, the effect of the present invention is gradually decreased.

The existence of such dye-reserving layer 1 can be confirmed from the fact that, when the fibers of the present invention are dyed with an anionic dye, especially with a dye having more than three sulfonic acid groups, e.g. Drimarene Brilliant Red X-2B (a reactive dye produced by Sandoz) and are observed under a microscope, the fibers are dyed only from the cut ends.

The dye-reserving layer 1 is non-dyeable with anionic dyes because the amino groups in that layer of the hydrophobic fiber are blocked by covalent bonds. However, in reality, while some dyes cannot substantially pass through the dye-reserving layer, another can pass through that layer with comparative ease, unlike in the case of hydrophobic fibers which have completely been rendered non-dyeable or low dyeable to the core of the fibers. Thus, among anionic dyes, those having a single sulfonic acid group can pass through the dye-reserving layer 1 to dye even the core of the fibers sufficiently. However, with the increase in the number of sulfonic acid groups in the dye it becomes more and more difficult for the dye to pass through the dye-reserving layer and therefore the fibers do not become dyed. By the use of this phenomenon, the fibers of this invention can be dyed to have a multicolored effect. Of course it is possible to use another type of dye in combination, for example disperse dyes. Moreover, dyeing with anionic dyes gives dyed articles of bright color and having good fastness to wet treatment and light.

It is also possible to obtain more complex multi-colored effects when the dye-reserving layer is formed partly along the length of the hydrophobic fibers. The dyeability can be also varied in various ways by changing, for example, the thickness of the dye-reserving layer, the density of blocking of amino groups, etc. Also, very attractive multicolored effects can be obtained by the combination of dyes having different numbers of sulfonic acid groups.

10 The fibers of the present invention are suitable for producing yarn or cloth of a pepper-and-salt effect by the combination with other hydrophobic fibers containing amino groups having different dyeability or with fibers of other types. Especially the use of the fibers of

15 the present invention in articles of interior decoration, such as carpets, gives multicolored products of charming effects that have not been obtained in conventional articles.

20 Generally, the hydrophobic fibers of the present invention can be produced by reacting a compound having groups capable of linking to amino groups in the fibers to form covalent bonds, with only the surface portion of the fiber. Such compounds having groups

25 capable of forming covalent bonds with amino groups are preferably colorless or white compounds having reactive groups capable of reacting with amino groups, such as halotriazinyl, halopyrimidinyl, haloquinoxalyl, haloacrylamido, vinylsulfo groups, etc., or any other

30 groups that can produce these groups. However, colored compounds may be also used for the purposes of the present invention. Also suitable are compounds having anionic groups, for example, sulfonate, carboxylate, sulfate, phosphate groups, etc., besides the highly reactive groups capable of reacting with amino groups.

35 More specific examples of such compounds are those having the following general formula:



55 or  $\text{Hal}-\text{CH}=\text{C}(\text{Hal})-\text{CONH}-\text{Y}-(\text{A})_n$  where  $\text{Hal}$  is F, Cl or Br,  $\text{Z}$  is  $-\text{X}-\text{Y}-(\text{A})_n$ ,  $\text{B}$  is H, Cl or F,  $\text{X}$  is  $-\text{O}-$ ,  $-\text{S}-$  or  $-\text{NR}$ ,  $\text{Y}$  is an  $(n+1)$ -valent substituted or non-substituted an aromatic or aliphatic group,  $\text{A}$  is anionic group,  $n$  is 0 or a positive integer,  $\text{M}$  is H, alkali metal or ammonium, and  $\text{R}$  is H or a lower alkyl group.

60 The hydrophobic fibers containing amino groups include polyamide fibers, such as nylon-6, nylon-66; protein-acrylonitrile graft copolymer fibers such as Chinon (produced by Toyobo Co.); fibers of polyesters, polyurethanes, polyacrylonitrile, polypropylene, etc. which have been copolymerized, graft copolymerized or mixed with a compound having an amino group, for example, aminoalkyl acrylate, etc. Among them, polyamide fibers are most preferable.

The fiber to be treated with the above mentioned compound is usually in the form of fibers, filaments, yarn, but sometimes the treatment may be carried out

in respect of the fibers in the form of woven fabrics, knitted fabrics, non-woven fabrics, or paper.

There are various methods for reacting the surface portion of the fiber with the compound having groups capable of linking to amino groups to form covalent bonds.

One of such methods is to apply the dye-reserving agent to the fibers in a mist-like state, in a manner as shown in FIG. 2, wherein the numeral 3 indicates a means for applying a dye-reserving agent to the fiber *a*. The reference numeral 4 indicates the main body of the treating apparatus, and the reference numeral 5 designates a supply pipe of high pressure gas. The filaments *a* to be treated are given the dye-reserving agent at low temperature on the surfaces by the dye-reserving agent applicator 3 and then fed into the treating apparatus 4 through supply rollers 6,6'. Since the inlet 7 of the main apparatus 4 is narrowed and the high pressure gas supplied from the high pressure gas supply pipe 5 spurts out from the gas outlets 8,8' downwardly as a jet stream, the filaments *a* are drawn into the apparatus 4. The filament passage in the apparatus 4 is expanded sharply at the part 9, so that the jet stream turns into a violent turbulent stream therein. At this time, the filaments *a* are also violently vibrated to be opened, and the treating agent partly covering the surfaces of the filaments *a* leaves the filaments and floats in the form of mist to completely cover only the surface layer of the filaments again. The filaments having this surface deposit of the reserving agent are then dried by a heater 10 positioned at the lower part of the treating apparatus where the reaction on the filament surfaces is completed. The surface-treated filaments are taken-out by delivery rollers 11,11', and wound on a winding roller 12. If a compressed hot air is used as a high pressure gas, the heater 10 is not always necessary.

In the above mentioned method, the dye-reserving agent may be directly supplied at the inlet 7 of the treating apparatus or at the spreading part 9. If desired, the agent may be contained in the high pressure gas. The filaments are not necessarily required to be non-twisted yarn but may be soft-twisted yarn of less than 100 T/m.

Another example of treatment is that, an article to which the dye-reserving agent has been applied is squeezed and dried at low temperature and then subjected to heat treatment to fix the agent.

A further example of treatment is that unstretched filaments to which the dye-reserving agent has been applied is dried and then stretched to fix the agent by the heat developed by the stretching, or is stretched under heating to fix the agent.

In the above mentioned last two methods, it is preferable that the article under treatment should not be brought to a temperature higher than 50°C. before drying. If the article is raised above that temperature, the dye-reserving agent may penetrate into the core of the fibers and therefore the fibers of the present invention cannot be obtained. When the temperature is raised after drying, the dye-reserving agent reacts with the amino groups on the fiber surfaces and is fixed, so that it does not diffuse into the core of the fibers.

The dye-reserving agent may be used as an aqueous solution or an organic solvent solution. However, it is preferable to use it as an aqueous dispersion with suitable adjustment of the concentration and (wet) pick up such that the fibers take up 0.01 to 0.5% by weight of the agent based on the weight of the fibers.

When the dye-reserving agent is used in the form of an aqueous solution, the reactive groups in the agent may react with water and are hydrolyzed, so that the reactivity with amino groups is gradually lowered.

Therefore, in such case it is preferable to lower the water solubility of the agent, for example by maintaining the treating liquor at a low temperature or by modifying the sulfonic acid groups into the form of their salts or free acid having slight water solubility or by adding a mineral salt such as sodium sulfate, sodium chloride, etc., so that the hydrolysis proceeds only from the surfaces of the dispersed particles and therefore the agent is kept stable.

The methods of forming a dye-reserving surface layer intermittently along the lengthwise direction of the fibers include (1) a method of applying the dye-reserving agent intermittently along the lengthwise direction of the fibers; (2) a method wherein after the agent is applied to the whole surfaces of the fibers and fixed at some parts of the surfaces, the dye-reserving agent on the other parts is removed; and (3) a method wherein after the dye-reserving agent is applied to the whole surfaces of the fibers and fixed, some parts of the surface layer are stripped off.

An example of the method (1) is that the travelling yarns are contacted intermittently with a dye-reserving agent-supplying roller. An example of the method (2) is that after the dye-reserving agent is applied and dried, some parts of the agent are fixed on the yarns or

fabrics and the yarns or fabrics are then washed to remove the agent in the other parts. A peculiar example of this method is that after the dye-reserving agent is applied to unstretched filaments and dried, the filaments are stretched in some parts and the dye-reserving agent is fixed to the filaments by the heat developed by the stretching. In this case since the filaments are formed into "thick-and-thin" yarn, the contrasting difference of color is further emphasized to produce an interesting effect. Among examples of the method (3)

is a method of pressing the fibers with a pair of gears, a method of scratching some parts of the fiber surfaces with an edge, a method of pressing some parts of the fibers with a hot roller, a method of passing the fibers through sands or glass powder, etc., a method of strongly pressing some parts of the fibers with engraved hot rollers, a method of strongly pressing the fibers superposed with rugged cloth as a lace or rugged paper, with hot rollers, etc.

The fibers thus obtained are dyed mainly with anionic dyes including ordinary acid dyes, metallized dyes, direct dyes, reactive dyes, etc., and any of such dyes can be used satisfactorily. As mentioned above, the dyeability of the fibers depends on the number of sulfonic acid groups contained in the dye. Examples of the

dyes containing a single sulfonic acid group are C.I. Acid Yellow 25, 29, 49, 64, 65, 110, 135, 159, 168, C.I. Acid Orange 116, 127, C.I. Acid Red 32, 57, 257, 266, 333, 334, C.I. Acid Violet 31, 41, C.I. Acid Blue 25, 27, 40, 41, 47, 62, 72, 78, 106, 129, 230, C.I. Acid

Green 83, C.I. Acid Brown 248, etc. Examples of the dyes containing two sulfonic acid groups are C.I. Acid Yellow 17, 38, 42, 44, 79, C.I. Acid Orange 33, C.I. Acid Red 37, 154, 157, 168, C.I. Acid Violet 48, C.I. Acid Blue 80, 112, 182, 203, C.I. Acid Green 27, 41, etc.

Examples of the dyes containing three or more sulfonic acid groups are C.I. Acid Red 145, C.I. Direct Red 95, C.I. Reactive Yellow 2, 12, C.I. Reactive Orange 2, C.I. Reactive Red 3, 4, 9, 12, 17, 56, C.I.

Reactive Blue 2, 5, 10, 52, etc.

The dyeing conditions may be those used for ordinary dyeing with anionic dyes. Preferred conditions are pH 4-7, about 100°C., and 30-60 minutes. At a lower pH, the effect of non-dyeability is weakened and staining by dyes having a larger number of sulfonic acid groups becomes noticeable.

The present invention is explained with reference to the following examples.

### EXAMPLE 1

Filament yarn of nylon-6 (1100 d/68 f), while travelling, was brought into contact with the surface of a rotating roller dipped in a bath consisting of



5 parts by weight

and disodium hydrogenphosphate  
water

2 parts by weight  
93 parts by weight

30



2 parts

so that the yarn could take up 3% by weight of the solution based on the weight of the fibers. The yarn was then introduced into a treating apparatus as shown in FIG. 2, while a jet stream of high temperature high pressure air at 190°C. and 4 kg/cm<sup>2</sup> was blown thereto so that the yarn was opened into individual filaments and at the same time crimp-processed. At this time, the solution of the dye-reserving agent which covered the surfaces of the fibers more or less unevenly was blown off into fine mist-like droplets by the high speed jet stream, and the mist then covered the filaments again uniformly and became fixed by reacting with the amino groups on the surfaces of the fibers.

The yarn thus treated and yarn similarly crimp-processed but not treated with the dye-reserving agent were formed into twisted yarn. A carpet was prepared from this twisted yarn and was dyed in a bath containing

C.I. Direct Red 95 1% o.w.f.  
and Ultra N-1 (pH adjusting agent produced by  
Mitsubishi Chemical Co.) 0.2 g/liter

at a liquor ratio of 1:50 and at a temperature of 100°C. for 60 minutes. The result was that the yarn treated with the dye-reserving agent was not dyed at all while the yarn not treated was dyed in deep scarlet.

Undyed cut pieces of the both yarns (treated and untreated) were prepared and dyed with the above-mentioned dye. The cross-section of each of them was observed. Both were dyed in quite the same depth of color. It was observed under a microscope, however, that the surface layer of the yarn treated with the dye-

reserving agent was not dyed. The thickness of the dye-reserving layer of the treated yarn was about 1 micron when observed by means of microscopic photographs of the cross-sections of the fibers.

5 The content of amino groups as a whole was 55 milliequivalent/kg fibers for the untreated yarn and 53 milliequivalent/kg fibers for the yarn treated with the dye-reserving agent. Thus, there was no substantial difference between the two since the surface layer of 10 which the amino groups were blocked was very thin.

### EXAMPLE 2

Filament yarn of nylon-6 (1100 d/68 f), while travelling, was contacted intermittently with the surface of a rotating roller dipped in a bath consisting of



2 parts

and disodium hydrogenphosphate  
water

96 parts

35 and immediately introduced into a treating apparatus as shown in FIG. 2 where it was treated as in Example 1. In this way, filament yarn was produced which had an intermittent thin dye-reserving layer (about 1 micron thick) formed evenly on the surface of the filaments.

40 The yarn was then formed into a carpet, which was dyed in a bath consisting of

|                     |                    |
|---------------------|--------------------|
| C.I. Acid Brown 248 | 1.2 % o.w.f.       |
| C.I. Acid Red 57    | 0.2 % o.w.f.       |
| C.I. Acid Blue 72   | 0.35 % o.w.f.      |
| acetic acid         | 2 % o.w.f.         |
| water               | and<br>the balance |

50 at a liquor ratio of 1:50, at a temperature of 100°C for 45 minutes.

The result was that the parts covered with the dye-reserving agent were dyed medium brown while the parts not covered with the agent were dyed deep brown, thus producing a two tone effect. The state of the parts covered with the dye-reserving agent and the state of the parts not covered therewith were quite the same as in Example 1.

### EXAMPLE 3

Threads of nylon filaments (1100 d/68 f) arranged in parallel at intervals of 2 mm. were brought into contact with the surface of a roller rotated and dipped in a bath consisting of



2 parts  
sodium acetate  
and water

2 parts  
96 parts

so that the threads could take up the solution. The threads were then squeezed with a metallic roller to a pick-up of 20% and dried gradually at 50°C. Initially, only water was evaporated at such comparatively low temperature and a film of a liquid high in the concentration of the dye-reserving agent was formed on the surfaces of the fibers. When the temperature was elevated to 150°C., the dye-reserving agent was reacted with the amino groups in the fibers and a dye-reserving layer was formed.

Thus treated filament yarn was twisted with filament yarn which had not been thus treated. The twisted yarn was dyed in an aqueous bath containing

C.I. Direct red 95      1 %  
and Ultra N-1      0.2 g/liter

at a liquor ratio of 1:50 at a temperature of 100°C. for 60 minutes.

The result was that, while the treated yarn was not dyed at all, the untreated yarn was dyed in a deep scarlet color.

The same twisted yarn was dyed in a bath containing

C.I. Acid Yellow 17      0.5 % o.w.f.  
Mylanthrene Brilliant Blue 3BLF  
(an acid dye produced by Althaus)  
and acetic acid      1 % o.w.f.  
0.5 % o.w.f.

40

at a temperature of 100°C. for 60 minutes. The result was that, while the untreated filament yarn was dyed green, the treated yarn was dyed blue. The cross-section of the treated filaments showed that the thickness of the dye-reserving layer was less than about 2 microns.

#### EXAMPLE 4

Five hundred threads of Exlan H type filaments (acid dye-dyeable acrylic fibers containing amino groups produced by Japan Exlan Company, Limited; 100 d/40 f) were arranged in parallel and were passed through a bath composed of



2 parts  
sodium acetate  
acetic acid  
water

1 part  
0.05 part  
the balance

and squeezed. Then, under similar conditions as in Example 3, a dye-reserving layer was formed on the surfaces of the fibers. The yarn thus treated and the yarn which was not passed through the dye-reserving agent bath but treated in the same manner in all other respects were woven into a fabric by using these two types of yarn alternately. The fabric thus obtained was dyed in a bath containing

10      C.I. Reactive Blue 10      2 %  
and Ultra N-1      1 g/liter

at a liquor ratio of 1:50 at a temperature of 100°C. for 60 minutes. The result was that the treated yarn remained white while the untreated yarn was dyed in a deep navy blue to obtain a dyed checked fabric. The cross-section dyeing of the treated filaments showed that the thickness of the dye-reserving layer was less than 2 microns on the average.

#### EXAMPLE 5

Chips of nylon-6 having a relative viscosity of 2.5 were melted and spun into filament yarn at a temperature of 260°C. and at a winding speed of 800 m/min. The filament yarn was made to take up the following treating liquor in an amount of 6% on the weight of the fibers from an oiling roller, and wound up.



(a)      3 %  
15 %  
5 %  
the balance.

To prepare the bath, sodium sulfate was dissolved in water and the solution was cooled to 20°C. The compound (a) was then added to the solution and dispersed by stirring with a high speed stirrer. This dispersion was mixed with the spinning oil which was then emulsified. The yarn was then stretched four times the initial length.

On the other hand, another sample of the same filament yarn was treated in the same way except that the oiling bath did not contain the compound (a), and was blended with the above-mentioned yarn which was treated with the compound (a). The resulting blended yarn was dyed with C.I. Direct Red 95 and yarn having a dotted effect of deep red and white was obtained. When dyed with C.I. Acid Yellow 135, the blended yarn was dyed in yellow colors with a slight difference in depth, and when dyed with a mixture of C.I. Direct Red 95 and C.I. Acid Yellow 135, the yarn represented an orange and yellow effect.

The above-mentioned bath was used continuously and the yarn spun after 5 days was examined for its shades after dyeing. It was found that the shades were substantially the same as those of the first day.

For the purpose of comparison, sodium sulfate which was used for decreasing the solubility of the compound (a) was removed from the bath and the bath was heated to 30°C. to dissolve the compound (a) completely. Spinning was run continuously for days while using this treating bath. After three days the shade of the dyed yarn changed definitely.

## EXAMPLE 6

Filament yarn of nylon-6, while travelling, was brought into contact with a roller rotated and dipped in a bath containing



and disodium hydrophosphate

0.5 %

and was then crimp-processed with a jet stream of high temperature, high pressure air at 180°C. and 4 kg/cm<sup>2</sup>. When the yarn was dyed with Drimarene Brilliant Red X-2B (a reactive dye produced by Sandoz), the dyeing took place from only the cut ends of the filaments. This 25 yarn was combined with yarn similarly crimp-processed but not treated with the dye-reserving agent, and dyed with a bath containing

C.I. Acid Red 35 (containing two sulfonic acid groups) 0.5 % o.w.f.  
and C.I. Acid Blue 40 (containing a single sulfonic acid group) 1.2 % o.w.f.

at a liquor ratio of 1:50 and at a temperature of 100°C. for 40 minutes. The modified yarn and the yarn of 40 ordinary dyeability were dyed blue and violet respectively. For the purpose of comparison, nylon-66 type 845 (Du Pont, deep dyeable) and type 846 (Du Pont, regular) were combined and dyed in the same way as mentioned above. However the multicolored effect was 45 insufficient, being bluish violet and reddish violet.

## EXAMPLE 7

Chips of nylon-6 having a relative viscosity of 2.5 were melted and spun into filament yarn at a spinning 50 temperature of 260°C. and a winding speed of 800 m/min. The yarn was made to take up a treating liquor composed of



in an amount of 6 % on the weight of the fiber from an oiling roller and wound up. This unstretched yarn was

stretched four times of the initial length. When the stretched yarn was dyed with Drimarene Brilliant Red X-2B, only the cut ends of the filaments were dyed. This yarn was combined with yarn treated in an oiling bath not containing the compound (b). When the combined yarn was dyed in a bath containing

|                                                                    |    |              |
|--------------------------------------------------------------------|----|--------------|
| C.I. Reactive Blue 10 (containing 3 sulfonic acid groups)          | 10 | 1.0 % o.w.f. |
| and C.I. Acid Yellow 135 (containing a single sulfonic acid group) |    | 0.3 % o.w.f. |

at a pH of 5.5 as in Example 1, the yarn was dyed yellow and deep blue.

## EXAMPLE 8

Filament yarn of nylon-6 (1100 d/64 f), while travelling, was applied with a treating liquor (1) composed of



and another treating liquor (2) composed of



each independently and intermittently along the length of the yarn and thereafter crimp-processed by compressed hot air jet of 180°C. and 4 kg/cm<sup>2</sup>.

When the yarn thus obtained was dyed with C.I. Acid Blue 80 in the ordinary way, the parts not given the treating liquor (1) and (2) were dyed deep blue, the parts given the treating liquor (2) were dyed light-medium blue, the parts given the treating liquor (1) were dyed light blue, and the overlapped parts of the treating liquor (1) and (2) remained white.

When the yarn was dyed with C.I. Acid Yellow 135, there was only a very slight difference in shade. When the yarn was dyed with a mixture of the two dyes, the above-mentioned parts were dyed blue green, green, yellow green and yellow, respectively, to produce a more complex effect.

When the yarn was dyed with the mixture of

|                                                               |       |
|---------------------------------------------------------------|-------|
| C.I. Acid Yellow 49 (containing a single sulfonic acid group) | 0.8 % |
|---------------------------------------------------------------|-------|

-continued

C.I. Acid Red 158 (containing 2 sulfonic acid groups) 0.5 %  
 and C.I. Reactive Blue 10 (containing 3 sulfonic acid groups) 0.3 %.

the parts given the treating liquor (1), the treating liquor (2), both liquor, and not given either of them were dyed reddish yellow, orange, yellow and deep brown, respectively.

## EXAMPLE 9

The following two kinds of treating liquor containing dye-reserving agents were applied to filament yarn of nylon-6 intermittently along the length of the yarn and were fixed by the method as shown in Example 1.



and



and water the balance.

When the yarn was dyed with C.I. Acid Blue 80, it was dyed deep blue, light blue, green and yellow.

A tufted carpet was produced from the above-mentioned treated yarn and was dyed with C.I. Acid Blue 80 in one-bath dyeing. The carpet showed the same effect of colors and in addition much higher bulkiness than that produced from yarn-dyed yarn.

## EXAMPLE 10

Nylon-6 was melt-spun and the yarn before winding was made to take up 6 % by weight of a liquor of the following composition.



The unstretched yarn, after being allowed to stand for 2 days in a room at a temperature of 20°C. and a relative humidity of 65 %, was stretched by a draw-twister. The stretching ratio was intentionally varied intermittently to produce thick-and-thin yarn (stretching ratio at thick parts, 1.8 times; thin parts, 4 times). After being washed with water, the yarn was dyed with C.I. Acid Yellow 29 (containing a single sulfonic acid group). Yarn having very contrasting colors was obtained, the thick parts being dyed deep and the thin parts, light.

## EXAMPLE 11

Deep dyeable nylon-66 yarn containing 72 milliequivalent/kg. fiber of amino groups was subjected to surface dye-reserving treatment according to the method as shown in Example 1. This filament yarn was plied with crimp-processed light dyeable nylon-66 having an amino group content of 37 m.eq./kg. fiber. The plied yarn was dyed in an aqueous solution containing 1 % of o.w.f. of C.I. Acid Yellow 49 (containing a single sulfonic acid group) at 100°C. for 45 minutes in the usual way. The result was that the dye-reserving treated yarn was dyed deeper than the light-dyeable yarn. However, when dyed with C.I. Acid Blue 80 (containing two sulfonic acid groups) in the same way as above, the dye-reserving treated yarn was dyed lighter than the light-dyeable yarn. Also, when dyed with C.I. Reactive Red 3 or C.I. Reactive Blue 10 (both containing three sulfonic acid groups) in the same way as above, the dye-reserving treated yarn was not substantially dyed. When the plied yarn was dyed with a combination of the above-mentioned dyes (each 0.5 % o.w.f.), it was dyed in various colors as follows:

|                                                                         | Dye-reserving<br>treated yarn | Light dyeable<br>yarn |
|-------------------------------------------------------------------------|-------------------------------|-----------------------|
| C.I. Acid Yellow 49<br>+ C.I. Acid Blue 80                              | greenish yellow               | bluish green          |
| C.I. Acid Yellow 49<br>+ C.I. Reactive Red 3                            | yellow                        | scarlet               |
| C.I. Acid Yellow 49<br>+ C.I. Reactive Red 3<br>+ C.I. Reactive Blue 10 | yellow                        | deep brown            |

## 45 What is claimed is:

1. Hydrophobic fibers having a dye-reserving layer only on the surface of each individual fiber, produced by a method which comprises subjecting hydrophobic fibers containing amino groups to the action of a turbulent gas stream to cause exposure of the individual filaments thereof, and simultaneously therewith depositing a dye-reserving agent in mist form on the fibers, and subsequently fixing the dye-reserving agent on the fibers by subjecting the resultant fibers to a dry heat treatment, to form said dye-reserving layer, said dye-reserving agent being a compound selected from the group consisting of compound of the formulae:



wherein Hal is fluorine, chlorine or bromine, Z is —NR-phenyl sulfonate, B is hydrogen, chlorine or fluorine and R is hydrogen or lower alkyl.

13

2. The hydrophobic fibers as claimed in claim 1 wherein the thickness of the dye-reserving layer is less than about two microns.
3. The hydrophobic fibers as claimed in claim 1 wherein the dye-reserving layer is present intermittently along the lengthwise direction of the fibers.
4. Polyamide fibers according to claim 1.

5. Polyamide fibers according to claim 1, said fibers being mixed with polyamide fibers not having the dye-reserved surface layer thereon.

6. The hydrophobic fibers as claimed in claim 1 wherein the dye-reserving agent is applied to the fibers, and the resultant fibers are subjected to the action of

14

the turbulent gas stream to form a mist of the dye-reserving agent which has been applied to the fibers, said mist then being deposited on the fibers.

7. The hydrophobic fibers as claimed in claim 1 wherein the gas used to form the turbulent gas stream contains the dye-reserving agent, or the dye-reserving agent is blown directly into the turbulent gas stream, thus forming the mist of the dye-reserving agent.

8. The hydrophobic fibers as claimed in claim 1 wherein the dye-reserving agent is a dihalotriazine.

9. The hydrophobic fibers as claimed in claim 8 wherein the dye-reserving agent is a dichlorotriazine.

\* \* \* \* \*

15

20

25

30

35

40

45

50

55

60

65

UNITED STATES PATENT OFFICE  
CERTIFICATE OF CORRECTION

Patent No. 3,926,548 Dated December 16, 1975

Inventor(s) Kazuo Moriyama, Takashi Iwato and Morihiko Ohno

It is certified that error appears in the above-identified patent and that said Letters Patent are hereby corrected as shown below:

In claim 1, after the structural formula following line 12, insert



Signed and Sealed this  
Second Day of May 1978

[SEAL]

Attest:

RUTH C. MASON  
Attesting Officer

LUTRELLE F. PARKER  
Acting Commissioner of Patents and Trademarks